

## UNITED STATES PATENT OFFICE

ROMAINE G. WALTENBERG, OF ROSELLE, HENRY EDWIN HOLBROOK, OF IRVINGTON,  
AND BERT BRENNER, OF ELIZABETH, NEW JERSEY, ASSIGNEES TO THE H. A. WILSON  
COMPANY, OF NEWARK, NEW JERSEY, A CORPORATION OF NEW JERSEY

## ALLOY

No Drawing.

Application filed March 6, 1931. Serial No. 520,708.

This invention relates to alloys and is concerned more particularly with novel alloys to be used primarily for such purposes as contact points in devices for making and breaking electrical circuits.

In electrical devices of the type described, for example, voltage regulators, numerous alloys have been used for contact points, such as alloys of platinum with about 30% by weight of iridium, and binary alloys of platinum metals including approximately equal percentages of platinum, iridium, osmium, rhodium, ruthenium, and palladium. Such alloys, however, with the exception of platinum-palladium and platinum-rhodium with about 50% of rhodium by weight are subject to the important disadvantage of being unworkable by swaging, rolling or drawing. All these alloys, therefore, have to be machined or ground to the desired shape, and this necessitates difficult and expensive operations in the fabrication of the alloys to commercial forms, such as contact points.

The present invention is accordingly directed to the provision of alloys particularly useful for contact points which give better results in service than the alloys now commonly used and which are workable by swaging, rolling, and drawing, so that the contact points and other articles can be made from them without the expensive grinding and machining operations heretofore required.

We have found that the desired results may be obtained by employing iridium as the principal constituent of the alloys, using that metal in amounts greatly in excess of present practice. Alloys containing from 70% to 90% by weight of iridium with the remainder made up of one or more of the metals platinum, palladium, rhodium and ruthenium fulfill the requirements mentioned, although it was to be expected from the prior work done in this field, that an increase in the amount of iridium would make working more difficult. Our experiments have made clear that this is not the case and in addition to improved workability, an alloy containing 70 to 90% iridium with the remainder made up of one or more of the metals platinum, palladium, rhodium and ruthenium is of greater stability when used for contact purposes, the surface does not readily become oxidized or corroded, loss of the contact material due to mechanical wear or vaporization is reduced, and building up of one point by transfer thereto of material from the other is also lessened.

A superior alloy of the type described is one which consists of 80% iridium and 20% platinum by weight, although the proportions of the ingredients may be varied within the range mentioned.

What we claim is:

1. An alloy containing iridium to the amount of about 70% and the remainder made up of one or more of the metals platinum, palladium, rhodium, and ruthenium.
2. An alloy containing iridium varying from about 70% to 90% and the remainder made up of one or more of the metals platinum, palladium, rhodium, and ruthenium.
3. An alloy containing approximately 80% iridium and the remainder platinum.
4. An alloy containing iridium to the amount of about 70% to about 90% and the remainder platinum.
5. An alloy containing iridium to the amount of about 70% to about 90% and the remainder rhodium.
6. An alloy containing iridium to the amount of about 70% to about 90% and the remainder palladium.

In testimony whereof we affix our signatures.

ROMAINE G. WALTENBERG.  
HENRY EDWIN HOLBROOK.  
BERT BRENNER.

85

90

95

100